

# UNITED STATES PATENT OFFICE.

ARTHUR ARENT, OF DES MOINES, IOWA, ASSIGNOR TO ARTHUR ARENT LABORATORIES, INC., OF DES MOINES, IOWA, A CORPORATION OF IOWA.

## ART OF PROTECTIVELY TREATING WOOD AND THE LIKE.

1,418,609.

Specification of Letters Patent. Patented June 6, 1922.

No Drawing.

Application filed November 14, 1919. Serial No. 338,088.

To all whom it may concern:

Be it known that I, ARTHUR ARENT, a citizen of the United States, residing at Des Moines, in the county of Polk and State of 55 Iowa, have invented certain new and useful Improvements in the Art of Protectively Treating Wood and the like; and I do hereby declare the following to be a full, clear, and exact description of the invention, such 10 as will enable others skilled in the art to which it appertains to make and use the same.

This invention relates to the art of protectively treating wood and the like; and it 15 comprises a process of preserving or protectively treating such material by applying thereto a non-aqueous solution, more particularly a solution in a tarry solvent such as creosote or the like, of a metal compound 20 which is hydrolyzable to yield a substantially water-insoluble compound of the metal. The invention also comprises the novel products resulting from the process.

The invention is particularly applicable 25 to the treatment of wooden piles for protection against the ravages of the teredo or marine borer, and for the sake of a concrete example embodying the principles of the invention, the application of the process to 30 treatment of piling will be described, hereinafter in detail. It is to be understood, however, that the invention is not limited to this specific use, but is also applicable to the treatment of fibrous materials generally, 35 such as wood, wood pulp, paper, canvas, duck, textile fabrics generally, etc.

This application is in part a continuation 40 of my copending application Serial No. 306,928, filed June 26, 1919.

The difficulty of protecting piling against 45 the attacks of the marine borer is well known, and so far as I am aware no thoroughly satisfactory solution of the problem has heretofore been available. The impregnation 50 of such piling with tarry materials alone, such as creosote or the like, does not give the requisite protection. It has been proposed heretofore to incorporate in the impregnating material metallic salts having 55 distinct toxic properties; but such proposed methods have not met with a high degree of

success, largely for the reason that the salts employed were dissolved out of the piling by the sea water and the piling thus left exposed to the attacks of the borer.

In accordance with the present invention, the described difficulties have been overcome and certain novel advantages obtained by treating wooden piles with a non-aqueous solution of a metal compound which, upon 60 exposure to moisture or water is hydrolyzed with the production of a metal compound substantially insoluble in water. In piles thus treated, the metal of the toxic compound employed is tenaciously retained in 65 insoluble combination even after long exposure to and contact with water and continues to exercise its protective function by virtue of its toxic action on borers and other organisms against which protection is required.

In practicing the process of the present invention, I have found the use of an antimony salt to offer special advantages as a toxic agent; and among the antimony salts 75 available, a chlorid of antimony, most desirably antimony trichlorid, has proved of particular value for impregnation of wooden piles to be submerged in sea water. Antimony trichlorid is soluble in a number 80 of non-aqueous solvents among which may be mentioned alcohol, amyl acetate, carbon tetrachlorid and other carbon chlorids, carbon bisulfid, etc. By non-aqueous solvent is here meant a solvent which is composed 85

wholly or largely of a liquid other than water. If water is present at all in the solvent employed in practicing the process of the invention, it should be present in proportions insufficient to cause substantial hydrolyzation or decomposition of the salt employed and consequent deposition of an insoluble oxid or basic salt during treatment of the article or material to be impregnated, I have also found that antimony trichlorid 95 can be dissolved directly in tarry materials which are either liquid at ordinary temperatures or can be readily liquefied upon heating; and among such tarry materials creosote is especially advantageous for present 100 purposes.

In treating wooden piles according to the

process of the invention, anhydrous antimony trichlorid may be dissolved directly in creosote, with or without the aid of heat. The proportions of antimony trichlorid to be used may vary considerably in practice, but I have found that creosote containing about two pounds of antimony trichlorid per gallon is very effective. Instead of dissolving the antimony trichlorid directly in the creosote, it is also possible first to dissolve the trichlorid in a non-aqueous solvent vehicle such as carbon tetrachlorid, amyl acetate, or the like, and then to mix this solution with creosote in the required proportions. The solution of antimony trichlorid in creosote, however prepared, may be employed for impregnation of piling by any well known or suitable method, the particular way in which this impregnation is effected forming no part of the present invention.

Piles treated with the described solution of antimony trichlorid in creosote are substantially proof against destructive attack by the teredo or other pests of this character even after prolonged submersion in sea water. Such part of the original content of antimony trichlorid as eventually comes into contact with water as a result of prolonged submersion is simply hydrolyzed with the production of insoluble basic chlorides or oxids of antimony, which latter are therefore not washed out of the wood but remain there permanently as protective toxic agents. Among other obvious applications of the broad principles of the invention may be mentioned the treatment of lumber, shingles, and the like, with creosote or other suitable non-aqueous vehicle solvent containing antimony trichlorid. Even where materials of this kind are not exposed to the attacks of borers, treatment in accordance with the invention offers great practical advantages because of the fact that such materials can be rendered practically non-inflammable in this manner.

While the use of antimony trichlorid has been particularly referred to in illustrating a practical embodiment of the novel process, it is entirely feasible to make use of other salts of antimony, such as other halids, the sulfate, etc., and also to make use of similar compounds of other metals which in a general way behave in an analogous manner when exposed to the action of moisture or water, and which are also soluble in non-aqueous vehicles of the general character described. By way of example may be mentioned compounds of other metals of the antimony group, that is, compounds of bismuth and arsenic, as well as compounds of tin. Compounds of all these various metals may be dissolved in one or another of the various non-aqueous solvent vehicles above

mentioned or available, or in mixtures of said solvents, and in this condition may be employed for impregnation of wood or woody materials broadly, in a manner analogous to that already described for impregnation of wooden piles with creosote containing an antimony salt.

In practice, however, I have found the employment of an antimony salt, especially antimony trichlorid, to give most satisfactory results. A salt of this type is substantially instantly decomposed upon contact with water to yield an insoluble product.

What I claim is:

1. The process of protectively treating woody materials which comprises applying thereto a tarry solution of a toxic and fire-retardant metal compound hydrolyzable to yield a water-insoluble compound of the metal.

2. The process of protectively treating woody materials which comprises impregnating said materials with a tarry solution of a compound of a metal of the antimony group.

3. The process of protectively treating woody materials which comprises impregnating said materials with a non-aqueous solution of antimony trichlorid.

4. The process of protectively treating wooden piles which comprises impregnating the same with a non-aqueous solution of a compound of a metal of the antimony group.

5. The process of protectively treating wooden piles which comprises impregnating the same with tarry material containing dissolved therein a metal compound hydrolyzable to yield an insoluble compound of the metal.

6. The process of protectively treating wooden piles which comprises impregnating the same with tarry material containing dissolved therein a hydrolyzable compound of a metal of the antimony group.

7. The process of protectively treating wooden piles which comprises impregnating the same with tarry material containing an antimony salt.

8. The process of protectively treating wooden piles which comprises impregnating the same with tarry material containing antimony trichlorid.

9. The process of protectively treating wooden piles which comprises impregnating the same with creosote containing antimony chlorid dissolved therein.

10. The process of protectively treating woody material which comprises impregnating the same with a non-aqueous solution of a toxic and fire-retardant metal compound hydrolyzable to yield a water-insoluble compound of the metal.

11. As a new article of manufacture, woody material impregnated with tarry

matter carrying a compound of a metal of the antimony group.

wooden pile impregnated with creosote containing antimony chlorid.

12. As a new article of manufacture, woody material impregnated with tarry matter carrying an antimony compound.

15. As a new article of manufacture, a wooden pile impregnated with tarry matter containing antimony trichlorid.

13. As a new article of manufacture, a wooden pile impregnated with tarry matter carrying an antimony salt.

In testimony whereof I hereunto affix my signature.

14. As a new article of manufacture, a

ARTHUR ARENT.